

## UNITED STATES PATENT OFFICE

GEORGE F. DORAN, OF WORCESTER, MASSACHUSETTS

## REFINING AND PURIFICATION OF METALS

No Drawing.

Application filed March 14, 1931. Serial No. 522,789.

This invention relates to the refining and purification of metals.

The object of the invention is to improve the physical characteristics of metals and alloys by treating the same, while in molten condition, with a salt of permanganic acid. Such salts are potassium permanganate, sodium permanganate and their equivalents.

Manganic compounds, such as  $K_2MnO_4$ , may also be used for said purpose.

A further object of the invention is to increase the resistance of nickel and nickel alloys to tarnish or corrosion, and to close grain the metal and increase the tensile strength of same.

Manganese and oxides of manganese are known to have been used for the treatment of molten metals. I have found that potassium permanganate acts in a manner entirely different than metallic manganese and the oxides of manganese when incorporated with molten metal. For example, I have found that treatment of nickel silver, while in a molten state, with potassium permanganate increases the tensile strength of nickel silver and also increases its resistance to tarnish in a strikingly unexpected manner in contrast to the results obtained by the treatment of the same metal with the oxides of manganese or manganese metal. I am not prepared to state the actual theory of the reaction, but I believe it is due to the liberation of nascent potassium and nascent manganese. I have tried the addition of potash and also potassium alone as a purifier of nickel silver, and have also tried the addition of separate quantities of potassium and manganese, but I have been unable to obtain by the treatment of the metal with such substances the novel results obtained by the use of potassium permanganate. I have also experimented with the various salts and oxides of manganese, other than the permanganates, in the treatment of metals, and I have found that they do not impart to the metal the capacity to resist tarnish or corrosion which is imparted to the metal by the addition of permanganate.

I prefer to treat the molten metal with the potassium permanganate in the presence of a little carbon. However, the addition of car-

bon may be omitted where carbon is present in the crucible or raw materials, as the potassium permanganate under these conditions, when added to a molten metal mixture, acts as a powerful deoxidizer and purifies the metal thoroughly. As there is no water present, the permanganate salt cannot act as an oxidizing agent. It is my belief that the usual oxides of manganese, when added to molten metal, do not break down entirely and that they consequently leave the metal permeated with oxides, whereas the treatment of the molten metal with potassium permanganate in the presence of carbon will have a maximum deoxidizing effect upon the molten metal and possibly will form complex inner anhydrides. This theory is based upon the exceedingly short time required for the reaction between the molten metal and the permanganate to take place, whereas when other oxides are added to the molten metal, a longer time must elapse before any reaction will take place.

The following is an example of how my invention may be carried out:

A nickel silver alloy was made up by mixing 60 pounds of ingot copper with 20 pounds of nickel and melted in a graphite crucible. When these metals were thoroughly mixed, 20 pounds of zinc were added. Potassium permanganate in the proportion of one per cent. by weight of the metals was then added and well mixed with the melt just before the latter was poured into moulds. The time required for the permanganate to act upon the melt was just a few seconds. The metal treated showed an increase of 33% in tensile strength over the same metal not treated with permanganate. It was found that the untreated metal was readily corrodible by weathering, whereas the metal which had been treated with permanganate was highly non-corrosive.

Obviously, the permanganate might be added to the molten metal while in transit from the furnace to the molds or even after the metal has been poured into the molds.

The following comparative results have been obtained by the treatment of nickel sil-

ver with permanganate, manganese dioxide, and manganese, respectively:

| 5  | Treatment               | Tensile strength        |                         | Liver of sulfur corrosion test |
|----|-------------------------|-------------------------|-------------------------|--------------------------------|
|    |                         | Bar form                | Sheet form              |                                |
|    | 1% permanganate.....    | <i>Pounds</i><br>55,000 | <i>Pounds</i><br>79,800 | No discoloration.              |
| 10 | 1/2% manganese dioxide. | 35,400                  | 65,000                  | Tarnished.                     |
|    | .3% metallic manganese. | 36,999                  | 67,999                  | Do.                            |

15 The quantity of potassium permanganate to be added to the molten metal is preferably from  $\frac{1}{2}\%$  to 1% of the weight of the metal treated. However, it may be varied from a much smaller amount, say .1 per cent., to a much greater amount, say 5 per cent., as desired.

20 My permanganate treatment, when applied to steel, has produced excellent results as to resistance to corrosion and closing of the grain of the metal. My invention is applicable to steel, iron, and all non-ferrous metals, such as white metal, etc.

25 The addition of carbon is not always necessary, since some metals contain carbon as an impurity and melting crucibles often are of a carbonaceous nature. If carbon be added, the amount of same can be varied in proportion to the permanganate, although an excess of it is not harmful.

I claim as my invention:

30 1. A process of refining molten metal which comprises adding thereto potassium permanganate and carbon in amount sufficient to produce a deoxidizing reaction.

35 2. A process of scavenging non-ferrous metal which comprises simultaneously adding to the molten metal a small quantity of potassium permanganate and carbon.

40 3. A process of refining nickel-containing non-ferrous metal which consists in adding to the metal while in melted state a quantity of dry potassium permanganate in the proportion of from one-half per cent. to one per cent. of the molten metal and carbon.

45 4. A process of increasing the tensile strength and resistance to tarnish of non-ferrous metal, which consists in adding to the metal while in molten condition carbon and a dry salt of permanganic acid, and casting the metal immediately thereafter.

50 5. A process of deoxidizing molten non-ferrous metal, which consists in adding to the metal while in molten state a mixture of potassium permanganate and carbon, the carbon being present in amount sufficient to produce a deoxidizing action.

55 6. A process of refining nickel silver to increase its tensile strength and its capacity to resist tarnish which consists in adding to same while in a molten state a quantity of potassium permanganate of approximately one per cent. by weight of metal treated, si-

multaneously with sufficient carbon to produce a deoxidizing reaction.

In testimony whereof I have hereunto set my hand.

GEORGE F. DORAN.

70

75

80

85

90

95

100

105

110

115

120

12

1